

# UNITED STATES PATENT OFFICE.

JAMES RAMSEY SPEER, OF TRAPPE, MARYLAND.

## PROCESS OF MAKING IRON ALLOYS.

1,291,220.

Specification of Letters Patent.

Patented Jan. 14, 1919.

No Drawing.

Application filed May 3, 1915. Serial No. 25,458.

To all whom it may concern:

Be it known that I, JAMES RAMSEY SPEER, a citizen of the United States, residing at Trappe, in the county of Talbot and State of Maryland, have invented new and useful Improvements in Processes of Making Iron Alloys, of which the following is a specification.

My invention relates to an iron chromium nickel product that has the density and hardness equal to or greater than the various iron mixtures cast in or against a chill, and also has such homogeneity throughout the entire body of the casting, or roll, for example, that it has internally the same degree, or nearly the same degree, of hardness as the outside surface of the casting. For example, it is well known in the art that castings made from certain roll and chilling mixtures are greatly improved by having the wearing surface of the casting poured against a chill or chills either in the mold or forming a part of the mold from which the casting is made. My invention renders the use of a chill or chills unnecessary, because of the fact that the mixture of materials which I employ, produces such a hard resistance body throughout that any artificial or mechanical method of hardening the surface of the body of the casting is not essential.

Departing from the well known lines of manufacture in regard to chilling mixtures, I do not use any so-called chilling cast iron which is usually considered as having a high sulfur content. The charge from which I prefer to make my material consists approximately of equal parts of charcoal iron and low carbon steel scrap, with the addition of nickel and chromium in such proportion as to give the degree of hardness required from the use of the chromium, and the degree of toughness required from the use of the nickel. It is, of course, possible that a certain percentage of the nickel and chromium may be introduced in the manufacture through either the iron or the scrap. This, however, is immaterial. From my experience the chromium should run from .50 to 2%, and the nickel from .25 to 1% in the finished product.

In the mixture indicated above, I claim to have in combination, a relation of carbon to nickel and chromium which has not heretofore been employed. By the use of charcoal iron and low carbon steel scrap, the density of the resultant casting is very great. This density, in connection with the use of chromium and nickel, the effects of which are set forth in my patents, is indicative of a material having great hardness and toughness. The scleroscope test of my material produced as described herein, will run from 65 to 80 points of hardness above the degree of hardness in the highest class of so-called chilled cast iron metals. A micro-photograph of the structure of my material shows a maximum area of combined carbon and carbids contributing to great density and hardness.

I have also found that by annealing and heat treating my product, which eliminates the unnecessary internal strains, I get a maximum strength for an article of this class; tests showing close to 40,000 pounds per square inch tensile strength. This tensile strength, being greatly in excess of anything that is or has been produced in a chilled iron mixture, is of the greatest importance, especially in roll castings. The increased hardness as indicated by the scleroscope and tests of the material in service, show a degree of efficiency in and resistance to wear which has not heretofore been considered possible to obtain.

I claim—

1. The method of making an alloy highly responsive to heat treatment which consists in fusing together charcoal iron and low carbon steel, sufficient chromium to impart to the product the required hardness and nickel in a smaller quantity than the chromium and sufficient to impart to the alloy the required toughness, and then casting it into the desired article.

2. The method of making an alloy highly responsive to heat treatment which consists in fusing together approximately equal parts of charcoal iron and low carbon steel, sufficient chromium to impart to the product the required hardness and nickel in a smaller

quantity than the chromium and sufficient to impart to the alloy the required toughness, and then casting it into the desired article.

3. The method of making an alloy highly responsive to heat treatment which consists in fusing together approximately equal parts of charcoal iron and low carbon steel, chro-

mium from .50% to 2.00%, and nickel from .25% to 1.00%, and then casting it into the desired article.

Signed at New York, this 26th day of April, 1915.

JAMES RAMSEY SPEER.